

# United States Patent

Sugano et al.

[15] 3,652,416

[45] Mar. 28, 1972

## [54] OXIDE MAGNETIC MATERIALS

[72] Inventors: Izuru Sugano; Tsuneo Akashi; Tetsujin Matsubara; Yoshihiro Kenmoku; Taneaki Okuda, all of Tokyo, Japan

[73] Assignee: Nippon Electric Company, Limited, Tokyo, Japan

[22] Filed: Oct. 29, 1969

[21] Appl. No.: 872,094

### [30] Foreign Application Priority Data

Oct. 30, 1968 Japan.....43/79540

[52] U.S. Cl.....252/62.59, 252/62.61, 252/62.62, 252/62.63

[51] Int. Cl. ....C04b 35/38

[58] Field of Search .....252/62.59, 62.61, 62.62, 62.63

[56]

### References Cited

#### UNITED STATES PATENTS

|           |         |                   |           |
|-----------|---------|-------------------|-----------|
| 3,415,751 | 12/1968 | Hirota et al..... | 252/62.59 |
| 3,492,236 | 1/1970  | Ross .....        | 252/62.59 |

Primary Examiner—Daniel E. Wyman

Assistant Examiner—J. Cooper

Attorney—Sandoe, Hopgood and Calimafde

[57]

### ABSTRACT

Manganese-zinc ferrites are provided consisting essentially of manganese oxide, zinc oxide and iron oxide and small but effective amount of stannic oxide and lithium oxide ranging up to about 3.2 percent by weight of stannic acid and up to about 0.125 percent by weight of lithium oxide.

3 Claims, 18 Drawing Figures

SHEET 1 OF 8



INVENTORS  
 IZURU TSUNEO SUGANO  
 AMASHI  
 TETSUJIN MATSUBARA  
 YOSHIHIRO KENMOKU  
 TANEAKI OKUDA  
 BY

Sandoe, Hopgood & Calimafde  
 ATTORNEYS

PATENTED MAR 28 1972

3,652,416

SHEET 2 OF 8



INVENTORS  
IZURU SUGANO  
TSUNEO AKASHI  
TETSUJIN MATSUBARA  
YOSHIHIRO KENMOKU  
TANEAKI OKUDA

By  
Sandoe, Hotgood & Calmafde  
ATTORNEYS

PATENTED MAR 28 1972

3,652,416

SHEET 3 OF 8



FIG. 6



FIG. 5

INVENTORS  
IZURU SUGANO  
TSUNEO AKASHI  
TETSUJIN MATSUBARA  
YOSHIHIRO KENMOKU  
TANEAKI OKUDA  
Sando, Hopgood & Calma, Jr.  
ATTORNEYS

PATENTED MAR 28 1972

3,652,416

SHEET 4 OF 8



FIG. 7



FIG. 8

INVENTORS  
IZURU SUGANO  
TSUNEO AMASHI  
TETSUJIN MATSUBARA  
YOSHIHIRO KENMOKU  
TANEAKI OKUDA  
BY

Sandoe, Hopgood & Calmanoff  
ATTORNEYS

PATENTED MAR 28 1972

3,652,416

SHEET 5 OF 8



Sandoz, Hopgood & Calimafde  
ATTORNEYS



PATENTED MAR 28 1972

3,652,416

SHEET 6 OF 8



FIG. 12

INVENTORS  
IZURU SUGANO  
TSUNEO AKASHI  
TETSUJIN MATSUBARA  
YOSHIHIRO KENMOKU  
TANEAKI OKUDA

BY  
Sandol, Hopgood & Calmafield  
ATTORNEYS



FIG.14

INVENTORS  
 IZURU SUGANO  
 TSUNEO AKASHI  
 TETSUJIN MATSUBARA  
 YOSHIHIRO KENMOKU  
 TANEAKI OKUDA

Sandoe, Hopgood & Calma & de  
ATTORNEYS



FIG. 15



FIG. 16



FIG. 17

INVENTORS  
 IZURU SUGANO  
 TSUNEO AKASHI  
 TETSUJIN MATSUBARA  
 YOSHIHIRO KENMOKU  
 TANEAKI OKUDA  
 BY

Sandoe, Hoffgood & Calmire & de  
 ATTORNEYS

## OXIDE MAGNETIC MATERIALS

This invention relates to new oxide magnetic materials with greatly improved quality and hysteresis loss factors.

Manganese-zinc ferrites have found extensive applications as excellent soft magnetic materials for communications use in the frequency band near 100 KHz, and various improvements in magnetic properties have been attempted to cope with their diversified application fields. In keeping with the present-day rapid progress of communications equipment, miniaturization and high performance of magnetic cores have been in great demand, with the result that improvements in material and performance of ferrites themselves have become an important problem.

The addition of one, two or more kinds of additive or modifying agents to the manganese-zinc ferrite composition in a number of combinations has been attempted for the purpose of improving both quality and hysteresis loss factors. However, manganese-zinc ferrites with quality factors ( $\tan \delta/\mu$ ) and hysteresis loss factors ( $h_{10}$ ) less than  $2 \times 10^{-6}$  and 15 at 100 KHz, respectively, have hitherto not been attainable.

The quality factor and the hysteresis loss factor are defined according to the following equation:

$$R/\omega L = \tan \delta/\mu \cdot \mu e + h_{10} - (\mu^2/1000)^{3/2} \cdot (L/V)^{1/2} \cdot I,$$

wherein:

$R$  = effective resistance of core in ohms

$L$  = inductance of coil in henrys

$\mu$  = initial permeability of core

$\mu e$  = effective permeability of core

$V'$  = effective volume of core in cubic centimeters

$I$  = measuring current in amperes

It is an object of this invention to provide ferrites of the system  $MnO-ZnO-Fe_2O_3$  having markedly improved quality and hysteresis loss factors.

Other objects of the invention will more clearly appear from the following disclosure and the accompanying drawing, wherein:

FIGS. 1 to 18 illustrate the manner in which the magnetic properties of the ferrites are improved by this invention.

The present invention resides in the addition of stannic oxide ( $SnO_2$ ) and lithium oxide ( $Li_2O$ ), in combination to the manganese-zinc ferrite composition in amounts that effectively improves the loss characteristics of the ferrites, i.e., both the quality factor and the hysteresis loss factor.

Before describing in detail the subject matter of this invention, it will be noted hereinafter from Example 1 that a remarkable effect can be obtained for improvements in both the quality and the hysteresis loss factors when a compound of tin and a compound of lithium are added together to a manganese-zinc ferrite having a basic composition containing 55.9 mol percent  $Fe_2O_3$ , 38.0 mol percent  $MnO$ , and 6.1 mol percent  $ZnO$  as the main constituents so that the additives may ultimately take the form of  $SnO_2$  and  $Li_2O$ .

In Examples 2 through 6 also appearing hereinafter, it will be observed that the effect of combined  $SnO_2$  and  $Li_2O$  as additive agents remains substantially unchanged for manganese-zinc ferrites having different basic compositions from that mentioned in Example 1, and that there are optimum amounts of the additive agents and the allowable limits therefor for each basic ferrite composition.

In Example 7, it will be noted that the effect of the presence of  $SnO_2$  and  $Li_2O$  in the ferrite composition is markedly noticeable even when a special heat treatment is applied for improving magnetic properties as disclosed in Japanese patent application, No. 62961/1967.

Finally, in Example 8, it will also be noted that the effect of the addition of  $SnO_2$  and  $Li_2O$  per se remains substantially unchanged even when another combination of additives, such as  $CaO$  and  $SiO_2$ , is present in varying amounts in the manganese-zinc ferrite composition.

It will be understood, all the specimens used in the examples that follow were prepared according to the known sintering ferrite manufacturing method.

In producing the ferrite composition, iron oxide, manganese carbonate, zinc oxide, calcium oxide, and silicon oxide, together with the essential additive agents of this invention, i.e., stannic oxide and lithium carbonate, are individually weighed so as to obtain a predetermined composition and these compounds were mixed and pulverized for about 60 hours in a ball-mill using alcohol as a dispersion medium, followed by presintering the mixture for about 4 hours at about 800°C, pressing into a desired shape, firing for about 8 hours at about 1180°C in a nitrogen atmosphere containing 0.4 percent oxygen and then cooling. During cooling, the oxygen content in the nitrogen atmosphere is controlled.

All of the specimens in Examples 1 through 7 contained 0.06 wt. percent of calcium oxide and 0.02 wt. percent of silicon oxide, although not explicitly mentioned in each case. The effectiveness of the invention will be best understood by reference to the following examples.

## EXAMPLE 1

FIGS. 1 and 2 in combination demonstrate that the effect of  $Li_2O$  and  $SnO_2$  added together to a manganese-zinc ferrite having a basic composition of 38.0 mol percent  $MnO$ , 6.10 mol percent  $ZnO$ , and 55.90 mol percent  $Fe_2O_3$  is excellent insofar as improvements in the loss characteristics  $\tan \delta/\mu$  and  $h_{10}$  are concerned. An inspection of these graphs readily reveals the following: Both  $\tan \delta/\mu$  and  $h_{10}$  are markedly improved by the addition of  $SnO_2$  and  $Li_2O$  in small but effective amounts ranging from:

$$0.6 \text{ wt. \%} \leq SnO_2 \leq 2.7 \text{ wt. \%} \text{ and } 0 \text{ wt. \%} < Li_2O \leq 0.1 \text{ wt. \%}$$

Markedly improved materials meeting the two conditions  $\tan \delta/\mu < 1.0 \times 10^{-6}$  and  $h_{10} < 3$  at 100 KHz. heretofore not realized can be obtained.

## EXAMPLE 2

FIGS. 3 and 4 illustrate in combination the effect of  $Li_2O$  and  $SnO_2$  added together to a manganese-zinc ferrite having a basic composition of 36.0 mol percent  $MnO$ , 8.8 mol percent  $ZnO$ , and 55.2 mol percent  $Fe_2O_3$ . As is apparent, very good oxide magnetic materials meeting the two conditions  $\tan \delta/\mu < 1.0 \times 10^{-6}$ , and  $h_{10} < 3$  can be obtained by the addition of small but effective amounts of from 0.6 to 2.7 wt. percent  $SnO_2$  and from 0.01 to 0.1 wt. percent  $Li_2O$ . Such markedly improved magnetic properties have heretofore not been realized.

## EXAMPLE 3

FIGS. 5 and 6 illustrate in combination the effect of  $Li_2O$  and  $SnO_2$  added together to a manganese-zinc ferrite having a basic composition of 36.0 mol percent  $MnO$ , 9.5 mol percent  $ZnO$ , and 54.5 mol percent  $Fe_2O_3$ . As is apparent from these graphs, excellent oxide magnetic materials meeting the two conditions  $\tan \delta/\mu < 1.0 \times 10^{-6}$ , and  $h_{10} < 3$  at 100 KHz. are obtained by the addition of small but effective amounts of  $SnO_2$  and  $Li_2O$  in the ranges expressed as

$$2.0 \text{ wt. \%} \leq SnO_2 \leq 3.2 \text{ wt. \%}$$

$$0.01 \text{ wt. \%} \leq Li_2O \leq 0.06 \text{ wt. \%}$$

## EXAMPLE 4

FIGS. 7 and 8 indicate in combination the effect of  $Li_2O$  and  $SnO_2$  added together to a manganese-zinc ferrite having a basic composition of 34.0 mol percent  $MnO$ , 11.60 mol percent  $ZnO$ , and 54.4 mol percent  $Fe_2O_3$ . As is apparent from these graphs, the loss characteristics of the ferrites can be markedly improved by the addition of small but effective amounts of  $SnO_2$  and  $Li_2O$  expressed as

$$0.8 \text{ wt. \%} \leq SnO_2 \leq 2.3 \text{ wt. \%}$$

$$0 \text{ wt. \%} < Li_2O \leq 0.07 \text{ wt. \%}$$

and excellent oxide magnetic materials meeting the two conditions,  $\tan \delta/\mu < 1.2 \times 10^{-6}$  and  $h_{10} < 4$ , at 100 KHz. can be obtained.

These loss characteristics have not heretofore been realized by any known method.

#### EXAMPLE 5

FIGS. 9 and 10 indicate in combination the effect of  $\text{SnO}_2$  and  $\text{Li}_2\text{O}$  added together to a manganese-zinc ferrite having a basic composition of 34.0 mol percent  $\text{MnO}$ , 10.75 mol percent  $\text{ZnO}$ , and 55.25 mol percent  $\text{Fe}_2\text{O}_3$ .

As is apparent from these graphs, excellent oxide magnetic materials meeting the two conditions  $\tan \delta/\mu < 1.2 \times 10^{-6}$  and  $h_{10} < 4$ , heretofore have not been realized by known methods, can be obtained by the addition of small but effective amounts of  $\text{SnO}_2$  and  $\text{Li}_2\text{O}$  expressed as

$$\begin{aligned} 0 \text{ wt. \% } &\leq \text{SnO}_2 \leq 1.4 \text{ wt. \%} \\ 0 \text{ wt. \% } &\leq \text{Li}_2\text{O} \leq 0.06 \text{ wt. \%} \end{aligned}$$

#### EXAMPLE 6

FIGS. 11 and 12 indicate in combination the effect of  $\text{SnO}_2$  and  $\text{Li}_2\text{O}$  added together to a manganese-zinc ferrite having a basic composition of 32.0 mol percent  $\text{MnO}$ , 13.15 mol percent  $\text{ZnO}$ , and 54.85 mol percent  $\text{Fe}_2\text{O}_3$ . As is apparent, excellent oxide magnetic materials meeting the two conditions,  $\tan \delta/\mu < 1.3 \times 10^{-6}$  and  $h_{10} < 5$  at 100 KHz., can be obtained by the addition of small but effective amounts of  $\text{SnO}_2$  and  $\text{Li}_2\text{O}$  expressed as

$$\begin{aligned} 0.4 \text{ wt. \% } &\leq \text{SnO}_2 \leq 1.1 \text{ wt. \%} \\ 0.01 \text{ wt. \% } &\leq \text{Li}_2\text{O} \leq 0.05 \text{ wt. \%} \end{aligned}$$

As a result of conducting many experiments under various sintering conditions (such as disclosed in Japanese patent application No. 5507/1967 or when the sintering atmosphere is caused to change) other than that mentioned in the foregoing examples—that is, sintering for 8 hours at 1180°C in a nitrogen atmosphere containing 0.4 percent oxygen, the effect of combined stannic oxide and lithium oxide could be manifestly observed, although optimum composition ratios of  $\text{SnO}_2$  to  $\text{Li}_2\text{O}$  were subject to slight change.

The effect of the addition of  $\text{SnO}_2$  and  $\text{Li}_2\text{O}$  was substantially unaffected even if the sintered body was subjected to a heat treatment intended for improvements in magnetic properties such as disclosed in Japanese patent application No. 62961/1967.

An example for this is shown in Example 7 that follows.

#### EXAMPLE 7

FIGS. 13 and 14 illustrate respectively improvements in the loss characteristics  $\tan \delta/\mu$  and  $h_{10}$  of specimens of a ferrite having the same composition as in Example 1, i.e.,  $\text{MnO:ZnO:Fe}_2\text{O}_3 = 38:6.1:55.9$  mol percent and containing  $\text{Li}_2\text{O}$  and  $\text{SnO}_2$  as additive agents, the specimens being prepared, after sintering, by subjecting to a heat treatment for 32 hours at 250°C.

An inspection of these graphs readily reveals a marked degree of improvements in the loss characteristics  $\tan \delta/\mu$  and  $h_{10}$  due to the addition of small but effective amounts of  $\text{SnO}_2$  and  $\text{Li}_2\text{O}$  in the following ranges:

$$\begin{aligned} 1.0 \text{ wt. \% } &\leq \text{SnO}_2 \leq 2.9 \text{ wt. \%} \\ 0 < \text{Li}_2\text{O} &\leq 0.08 \text{ wt. \%} \end{aligned}$$

Thus excellent magnetic materials meeting the two conditions  $\tan \delta/\mu < 0.8 \times 10^{-6}$  and  $h_{10} < 3$  at 100 KHz. can be obtained.

The manganese-zinc ferrites used in this example contained 0.06 wt. percent  $\text{CaO}$  and 0.02 wt. percent  $\text{SiO}_2$  besides  $\text{SnO}_2$  and  $\text{Li}_2\text{O}$ . The effect of combined  $\text{SnO}_2$  and  $\text{Li}_2\text{O}$  per se was substantially unaffected when the amounts of addition of  $\text{CaO}$  and  $\text{SiO}_2$  were varied as will be evident from Example 8.

#### EXAMPLE 8

FIGS. 15 and 16 illustrate respectively graphs of  $\tan \delta/\mu$  and  $h_{10}$  of manganese-zinc ferrites having a basic composition of 38.0 mol percent  $\text{MnO}$ , 6.1 mol percent  $\text{ZnO}$ , and 55.9 mol percent  $\text{Fe}_2\text{O}_3$  and containing from 0 to 0.3 wt. percent  $\text{CaO}$

and from 0 to 0.04 wt. percent  $\text{SiO}_2$ . In contrast, FIGS. 17 and 18 illustrate respectively graphs of  $\tan \delta/\mu$  and  $h_{10}$  of these ferrites which contained 0.05 wt. percent  $\text{Li}_2\text{O}$  and 1.5 wt. percent  $\text{SnO}_2$  as another additive combination.

It will be apparent from the foregoing examples that a preferred manganese-zinc ferrite composition is provided consisting essentially of about 32.0 to 38.0 mol percent  $\text{MnO}$ , about 54.4 to 55.9 mol percent  $\text{Fe}_2\text{O}_3$  and the balance essentially  $\text{ZnO}$ , and containing about 0.01 to 0.1 weight percent  $\text{Li}_2\text{O}$ , about 0.4 to 3.2 weight percent  $\text{SnO}_2$ , less than about 0.3 weight percent  $\text{CaO}$  and less than about 0.04 weight percent  $\text{SiO}_2$ .

A comparison of these graphs readily demonstrates that the effect of addition of  $\text{SnO}_2$  and  $\text{Li}_2\text{O}$  per se is still conspicuous 15 under the co-presence of another additive combination  $\text{CaO}$  and  $\text{SiO}_2$  in varying amounts.

Any of the foregoing examples demonstrates that the addition of small but effective amounts of combined  $\text{SnO}_2$  and  $\text{Li}_2\text{O}$  are quite effective for improvements in the loss characteristics of the manganese-zinc ferrites.

The data of the figures together with the small but effective amounts of  $\text{SnO}_2$  and  $\text{Li}_2\text{O}$  added to the ferrites are summarized as follows:

| FIGS.     | MnO  | ZnO   | $\text{Fe}_2\text{O}_3$ | Wt. % $\text{Li}_2\text{O}$ | Wt. % $\text{SnO}_2$ |
|-----------|------|-------|-------------------------|-----------------------------|----------------------|
| 1 and 2   | 38.0 | 6.10  | 55.9                    | 0 < to 0.1                  | 0.6 to 2.7           |
| 3 and 4   | 36.0 | 8.8   | 55.2                    | 0.01 to 0.1                 | 0.6 to 2.7           |
| 5 and 6   | 36.0 | 9.5   | 54.5                    | 0.01 to 0.06                | 2.0 to 3.2           |
| 7 and 8   | 34.0 | 11.6  | 54.4                    | 0 < to 0.07                 | 0.8 to 2.3           |
| 9 and 10  | 34.0 | 10.75 | 55.25                   | 0 < to 0.06                 | 0 < to 1.4           |
| 11 and 12 | 32.0 | 13.15 | 54.85                   | 0.01 to 0.05                | 0.4 to 1.1           |
| 13 and 14 | 38.0 | 6.10  | 55.9                    | 0 < to 0.08                 | 1 to 2.9             |

Experiments were also conducted to determine the effective 35 limits in amounts of  $\text{SnO}_2$  and  $\text{Li}_2\text{O}$  added to many Mn-Zn ferrite compositions other than those indicated in these examples, covering a wide range as follows: 28 mol %  $\leq \text{MnO} \leq 40$  mol %; 51 mol %  $\leq \text{Fe}_2\text{O}_3 \leq 58$  mol %; balance  $\text{ZnO}$ .

Similar effects due to the addition of  $\text{SnO}_2$  and  $\text{Li}_2\text{O}$  were observed in such manganese-zinc ferrite compositions. The foregoing has established criteria for markedly improving the magnetic properties in reducing the values of  $\tan \delta/\mu$  and  $h_{10}$  to less than  $1.3 \times 10^{-6}$  and 5, respectively. The small but effective amounts of  $\text{SnO}_2$  and  $\text{Li}_2\text{O}$  to be added according to these criteria are less than about 3.2 wt. percent and less than 0.125 wt. percent, respectively, for example, from about 0.01 to 0.1 lithium oxide and from about 0.4 to less than 3.2 stannic oxide.

Experimental results have indicated it is difficult to meet these criteria through the addition of  $\text{SnO}_2$  and  $\text{Li}_2\text{O}$  in instances where the  $\text{MnO}$  content of the ferrite composition is considerably less than the above-stated minimum  $\text{MnO}$  content.

Although the present invention has been described in conjunction with preferred embodiments, it is to be understood that modifications and variations may be resorted to without departing from the spirit and scope of the invention as those skilled in the art will readily understand. Such modifications and variations are considered to be within the purview and scope of the invention and the appended claims.

What is claimed is:

1. A manganese-zinc ferrite composition consisting essentially of about 28 to 40 mol percent  $\text{MnO}$ , about 51 to 58 mol percent  $\text{Fe}_2\text{O}_3$  and the balance essentially  $\text{ZnO}$ , and further containing less than about 0.3 percent by weight of calcium oxide, and, less than about 0.04 percent by weight of silicon and small but effective amounts of less than about 3.2 percent by weight of stannic oxide and less than about 0.125 percent weight of lithium oxide, said amounts of stannic oxide and lithium oxide being sufficient to effect improvements in the values of the quality factor ( $\tan \delta/\mu$ ) and hysteresis loss factor ( $h_{10}$ ) of said composition, said ferrite composition being characterized by values of  $\tan \delta/\mu$  at 100 KHz. of less than  $1.3 \times 10^{-6}$  and  $h_{10}$  at 100 KHz. of less than 5.

2. The manganese-zinc ferrite of claim 1, wherein the lithium oxide ranges from about 0.01 to 0.1 percent by weight and wherein the stannic oxide ranges from about 0.4 to less than about 3.2 percent by weight.

3. A manganese-zinc ferrite composition consisting essentially of about 32.0 to 38.0 mol percent MnO, about 54.4 to 55.9 mol percent Fe<sub>2</sub>O<sub>3</sub> and the balance essentially ZnO, and

containing about 0.01 to 0.1 weight percent Li<sub>2</sub>O, about 0.4 to 3.2 weight percent SnO<sub>2</sub>, less than about 0.3 weight percent CaO and less than about 0.04 weight percent SiO<sub>2</sub>, said composition being characterized by values of tan δ/μ at 100 KHz. of less than  $1.3 \times 10^{-6}$  and  $h_{10}$  at 100 KHz. of less than 5.0.

\* \* \* \* \*

10

15

20

25

30

35

40

45

50

55

60

65

70

75